

## UNITED STATES PATENT OFFICE

2,035,894

## WETTING AGENT

Leopold Kahl, Berlin-Charlottenburg, Germany,  
assignor to Ruetgerswerke-Aktiengesellschaft,  
Berlin, Germany

No Drawing. Application July 8, 1933, Serial No.  
679,581. In Germany July 28, 1932

5 Claims. (Cl. 8—20)

This invention relates to wetting agents.

The wetting agents, hitherto employed in the mercerization of cotton, the function of which was to obtain rapid and uniform penetration of the fibres with concentrated soda lye, without preliminary bucking of the threads or fabrics, i. e. without first removing the dressing or size therefrom, are all characterized by the addition of mixtures of substances to the soda lye, which 0 in themselves are incapable of exerting wetting effects or only capable of exerting very slight wetting effects.

The mixtures, which it has hitherto been proposed to add to the soda lye in quantities of from 15 2 to 12%, include mixtures of low-boiling aliphatic alcohols with alcohols of higher molecular weight, mixtures of phenol or cresols with hydrated aromatic substances and mixtures of phenol or cresols and hydrated aromatic substances with aliphatic alcohols, aliphatic-aromatic alcohols or ketonic alcohols.

It has now been found according to the present invention that excellent wetting effects are obtained by employing only two components, comprising iso-amyl alcohol and phenol, cresols or xylenols or mixtures of the same which are poor in or free from  $\alpha$ -cresol.

With regard to the phenol, cresol or xyleneol components, it has been found that the  $\alpha$ -cresol 30 lowers the wetting action of the mixtures to an extraordinary degree. With regard to the alcohol components, it has been found that of all the alcohols the iso-amyl alcohol or the fermentation amyl alcohol chiefly containing this amyl alcohol is far superior to all the other alcohols 35 in its action. A mixture of only 2 parts of iso-amyl alcohol with 98 parts of practically  $\alpha$ -cresol-free phenol, cresol or xyleneol mixture or mixtures of the same yield wetting effects which become evident in a fraction of a second.

Whereas the upper limit of concentration for the lyes in the case of other wetting agents is as a rule as low as 32° Bé., since turbidities and separations occur at these concentrations, there 45 is practically no upper limit of concentration for the lyes, when employing  $\alpha$ -cresol-free phenols and a maximum of 2% of iso-amyl alcohol, calculated on the phenols.

The following examples illustrate the preparation 50 of a mercerizing bath according to the invention:

1. 2 parts by weight of iso-amyl alcohol are mixed with 98 parts by weight of practically  $\alpha$ -cresol-free phenol or cresol or xyleneol mixtures or a mixture of the same. 1,1 parts by weight of this mixture are added to the mercerizing lyes. 5

2. 2 parts by weight of iso-amyl alcohol are mixed with 98 parts by weight of phenol ( $C_6H_5OH$ ). 1-2 parts by weight of this mixture are added to the alkaline lye.

3. 2 parts by weight of iso-amyl alcohol are 10 mixed with 98 parts by weight of a technical, but  $\alpha$ -cresol-free xyleneol mixture, boiling for instance from 205° to 216° C. On adding this wetting agent in quantities of from 1 to 2% to a strong soda lye or potash lye a rapid and satisfactory wetting effect is obtained.

The iso-amyl alcohol may also be used in other quantities by weight, for example in quantities of from 3 to 10%, calculated on the total weight of the wetting agent. 20

The various components of the wetting agent are suitably mixed before adding it to the alkaline lye. To prepare the wetting agent in accordance with this invention, its components need not be 25 chemically pure.

By the term phenols as used in the present application, I mean the phenol  $C_6H_5OH$  as well as the mono- or poly-valent homologues of phenol, such as for example cresols, xyleneols etc. 30

What I claim is:

1. A composition for treating cotton fabrics and yarns which consists of an alkaline mercerizing solution and a mixture of iso-amyl alcohol and a phenol which is substantially free from  $\alpha$ -cresol. 35

2. A composition for treating cotton fabrics and yarns which consists of an alkaline mercerizing solution and a mixture of iso-amyl alcohol and a cresol substantially free of  $\alpha$ -cresol. 40

3. A composition for treating cotton fabrics and yarns which consists of an alkaline mercerizing solution and a mixture of iso-amyl alcohol and carboxylic acid substantially free from ortho-cresol. 45

4. A composition for treating cotton fabrics and yarns as claimed in claim 1, wherein the proportion of iso-amyl alcohol is more than 2%. 50

5. A composition for treating cotton fabrics and yarns as claimed in claim 1, characterized by using a mixture of several phenols.

LEOPOLD KAHL.